

removed, and the surfaces of the specimen left bright and shiny.

*Example 10*

A specimen of commercially pure magnesium taken from a rolled sheet of that metal was cleaned and left bright and shiny in 3 minutes by treatment at about room temperature in an aqueous solution containing 5 per cent sulfuric acid, 0.5 per cent malic acid, and 0.5 per cent oxalic acid.

These examples are given to indicate the compositions and methods of operating the solutions used in the practice of my invention, and it will be understood that variations in its practice are possible within the scope of the appended claims.

I claim:

1. The method of cleaning magnesium articles which comprises subjecting said articles to the action of an aqueous solution containing from about 1 to about 10 per cent sulfuric acid and a total of from about 0.5 to about 15 per cent of at least one aliphatic polybasic acid selected from the group consisting of oxalic, malic, citric, and tartaric acids.

2. The method of cleaning magnesium articles which comprises subjecting said articles to the action of an aqueous solution containing from about 2 to about 6 per cent sulfuric acid, and a total of from about 3 to about 5 per cent of at least one aliphatic polybasic acid selected from

the group consisting of oxalic, malic, citric, and tartaric acids.

5 3. The method of treating wrought magnesium articles in order to remove lubricants and other impurities therefrom and to produce a bright shiny surface thereupon, which method comprises subjecting said articles to the action of an aqueous solution containing from about 1 to about 10 per cent sulfuric acid and a total of from about 0.5 to about 15 per cent of at least one aliphatic polybasic acid selected from the group consisting of oxalic, malic, citric, and tartaric acids.

15 4. The method of cleaning magnesium articles and producing bright shiny surfaces thereupon which comprises subjecting said articles to the action of an aqueous solution containing from about 1 to about 10 per cent sulfuric acid and 0.5 to about 15 per cent citric acid.

5 5. The method of cleaning magnesium articles and producing bright shiny surfaces thereupon which comprises subjecting said articles to the action of an aqueous solution containing from about 1 to about 10 per cent sulfuric acid and 0.5 to about 15 per cent tartaric acid.

20 6. The method of cleaning magnesium articles and producing bright shiny surfaces thereupon which comprises subjecting said articles to the action of an aqueous solution containing from about 1 to about 10 per cent sulfuric acid and 0.5 to about 15 per cent oxalic acid.

MIKE A. MILLER.



June 23, 1942.

A. J. MUMMERT

2,287,051

PACKING RING

Filed Jan. 6, 1940

FIG. 1.



FIG. 2.



FIG. 3.



FIG. 4.



INVENTOR;  
ARDEN J. MUMMERT  
BY *J. Henry Kinealy*  
ATTORNEY